

1

2,934,396

## PROCESS OF DYEING HAIR WITH 5,6-DIHYDROXYINDOLE

Roger Charle, Soisy-sous-Montmorency, and Charles Pigerol, Saint-Ouen, France, assignors to Société Anonyme dite: Société Monsavon-l'Oreal, Paris, France, a corporation of France

No Drawing. Application January 27, 1958  
Serial No. 711,180

Claims priority, application France February 2, 1957

2 Claims. (Cl. 8—11)

This invention relates to methods and compositions for dyeing hair, particularly human hair, and like materials.

In our application No. 599,893 filed July 25, 1956, and now abandoned, we have described a process for dyeing hair and like fibers which consists essentially in (a) preparing an aqueous solution adjusted to an alkaline pH, containing 5:6-dihydroxy-indole and a reactant consisting of ammonia, an amine, an ammonium salt or an amine salt, (b) applying this solution to the hair or similar material to be dyed and rinsing the latter after a period of contact varying in accordance with the desired shade. In this way, relatively light shades ranging from light ash-blond to dark ash-blond are obtained for a standard period of contact of the order of from 20 to 30 minutes at room temperature, which period may be reduced by slight heating, for example, in the case of hair-dyeing, by means of a dry heat hood or a steam hood. It is furthermore possible, in accordance with the method of the aforesaid application, to obtain a more rapid development of the shade by adding to the dyeing solution, at the time of application, an oxidizing agent, such as sodium bromate, a persalt such as sodium perborate or ammonium persulphate, or simply hydrogen peroxide. There is to be noted that where an oxidizing agent is used it is necessary to make a well-balanced choice of the quantity added, a minimum quantity being necessary for a sufficiently rapid formation of the colored pigments, while an excess of this agent has the effect of more or less destroying said colored pigments intermediately formed and thus of reducing the depth of the final shade. As indicated in said application, it is possible to obtain dark shades closely comparable to the natural shades of the hair by operating in two steps, i.e. by first treating the hair with an alkaline solution of 5:6-dihydroxy-indole at room temperature for 15 to 30 minutes and then, after rinsing with water, applying to the hair a solution of an oxidizing catalyst.

It is an object of the present invention to provide a process for the dyeing of hair and like fibers by means of 5:6-dihydroxy-indole while still operating in two steps, wherein the 5:6-dihydroxy-indole solution applied in the first step, instead of being alkaline is either acid or neutral.

According to the present invention a process for dyeing live hair and like materials consists essentially in impregnating the hair or like material at room temperature with an aqueous solution of 5:6-dihydroxy-indole having a pH-value of at most 7, allowing the impregnation to proceed for about 5 to 60 minutes, blotting off the excess solution, and developing the shade in situ by applying an aqueous solution capable of inducing oxidation and/or polymerization of 5:6-dihydroxy-indole, the pH-value of which should be adjusted in accordance with the specific oxidizing agent to be used.

The pH-value of the aqueous 5:6-dihydroxy-indole solution to be applied in a first step for carrying out the invention may be obtained in various ways. For example, there may be employed an aqueous solution only containing the 5:6-dihydroxy-indole, with the exclusion of

2

any other reactant, the pH-value of such a solution being of course slightly acid. It is also possible to acidify this aqueous solution more or less strongly, for example by means of an inorganic acid, an organic acid, e.g. formic, acetic or monochloroacetic acid, or any compound containing at least one acid hydrogen atom.

The concentration of 5:6-dihydroxy-indole in the solution as applied to the hair or other material may vary within fairly wide limits. Generally it will be between 0.1% and 10% and preferably between 1% and 2% by weight of the solution. The term "aqueous solution" as employed here means any solution the principal solvent of which is water. It is of course possible, without departing from the scope of the invention, to use in the preparation of such a solution water alone or in admixture with water-miscible solvents, notably mixtures of water and ethyl alcohol or isopropyl alcohol or water and glycols or glycol ethers.

The aqueous solution of 5:6-dihydroxy-indole to be applied first may be prepared at the time of use. However, 5:6-dihydroxy-indole, like many other organic compounds, is relatively much more stable in acid or neutral medium than in alkaline medium and it is possible to have it prepared in advance in the form of any aqueous solution and, whenever desired, further to improve the stability of such a solution by adding thereto a small amount of a reducing agent, such as, for example, an alkali metal sulphite, bisulphite or hydrosulphite, this addition preferably being made first, i.e. before the 5:6-dihydroxy-indole is added. According to the present invention, the stability of aqueous solutions of 5:6-dihydroxy-indole may also be enhanced by adding thereto a small quantity, preferably 0.2% to 0.5%, of a sequestering agent, i.e. a compound capable of forming complexes with ions of alkaline-earth metals or of heavy metals, often existing as trace impurities. The sequestering agent may be, for example, ethylenediamine-tetracetic acid or one of its salts, such as that known under the trade mark "Trilon B."

When the aqueous 5:6-dihydroxy-indole solution has been in contact with the hair or other material for a period of 5 to 60 minutes the excess solution is blotted off, for example by pressing the hair in a towel.

The shade is then developed in situ by applying to the hair or other material an aqueous solution capable of inducing oxidation and/or polymerization of the 5:6-dihydroxy-indole.

The choice of this oxidizing agent, as also the length of time during which it should be maintained in contact with the hair or the material to be dyed, depends to some extent upon the final shade which it is desired to obtain. It is also possible to act upon the final shade by adjusting the pH of the developing solution to a pre-selected value, e.g. by including acid or alkaline materials therein.

In one method of carrying out the process of the invention there is used as oxidizing agent the oxygen of the ambient air, if desired ozonized. In such an embodiment the development of the shade, which amounts to the rapid fixing of the atmospheric oxygen by the hair or similar material impregnated with 5:6-dihydroxy-indole, is effected by applying in a second step as a developing medium an aqueous solution containing an alkalizing agent consisting preferably of ammonia, a basic ammonium salt such as ammonium carbonate or triammonium phosphate, or an organic amine. It is generally advantageous also to incorporate in this solution an oxidation catalyst which accelerates the process of fixing the oxygen of the ambient air, for example small quantities of a cobalt or manganese, salt, such as the sulphate or the lactate. The aqueous solution containing the alkalizing agent and, if desired, the oxidation catalyst is left in contact with the hair or similar material for 10 to 60

minutes as necessary for the penetration of the reactants. The hair is then rinsed clear with water and dried. The development of the shade, which is initiated by the alkalinization, may proceed for some time, this process then constituting a progressive dyeing process.

In a second method of carrying out the invention, there is applied in a second step, for the development of the shade, an aqueous solution of an oxidizing agent such as, for example, hydrogen peroxide, or an alkali metal or ammonium iodate, periodate or persulphate or an alkali metal salt of an N-chlorinated derivative of a sulphonamide. This solution is allowed to act for a period of time sufficient for the development of the shade, generally from 5 to 20 minutes, and the hair is then rinsed, shampooed, rinsed again and dried. The pH of this aqueous oxidizing solution, applied in the second place, may be adjusted to any desired value, either acid, neutral or alkaline, by the addition of any appropriate reactant, for example an inorganic or organic acid, a salt having an acid reaction, a buffer, a salt having a basic reaction or a base such as ammonia or an organic amine. The choice of the most suitable value depends mainly, but not solely, upon the nature of the oxidizing agent employed. If the latter is hydrogen peroxide, an alkali metal or ammonium iodate or periodate or an alkali metal salt of an N-chlorinated derivative of a sulphonamide, it is generally preferable to operate in a basic medium, whereas the operation is preferably carried out in an acid medium if the oxidizing agent is an alkali metal or ammonium persulphate. However, if the oxidizing agent employed is an iodate or a periodate, it is preferable not to operate at a pH-value lower than 3 and to avoid the use of a strong inorganic acid for adjusting the pH to the desired value.

Whatever the pH chosen for the development of the shade, the concentration of the oxidizing agent in the aqueous solution may be chosen between fairly wide limits, depending upon the desired shade and upon the own solubility of the specific oxidizing agent which is to be used. Generally speaking, the quantity of oxidizing agent to be employed corresponds to 0.5 to 10 g. per 100 cc. of solution, the volume of oxidizing solution to be employed being substantially the same as the quantity of dihydroxyindole solution.

When the oxidizing solution employed in the second step is acid or neutral, i.e. free from ammonia and organic amines, it is probable that the pigment formed results from the formation of the quinone corresponding to 5,6-dihydroxyindole. However analytical data has shown that if the oxidizing solutions are rendered alkaline by means of ammonia or an amine, the molecule of the pigment obtained contains nitrogen issuing from the ammonia or the amine employed. The same holds true when the oxidation is effected through the intermediary of ambient air and in the presence of ammonia or an amine, according to the first embodiment of the invention.

According to an accessory feature of the invention and whatever the specific embodiment to be dealt with, there can be advantageously added to the developing solution a quantity of a neutral, strongly ionized inexpensive electrolyte such as, for example, sodium chloride or sodium sulphate.

The dyeing process according to the invention may be carried out, not only by means of aqueous solutions as referred to above, but also by means of creams, pastes or jellies, the adjustment to the required consistency being effected by any method usual in hair dyeing.

The use of 5,6-dihydroxy-indole, under the above-defined conditions, constituting the object of the present invention may be combined with that of di- or triphenols capable of dyeing hair and other keratinous fibres at room temperature under analogous conditions such as those defined, for example, in our applications Nos. 709,479 and 709,602, both filed January 17, 1958.

The following examples will serve to illustrate the invention:

Example I illustrates the case where the development is effected in a basic medium and by oxidation in the ambient air, while the other examples illustrate cases where the development is effected by means of an oxidizing solution.

#### Example I

An impregnating solution having the following composition is prepared:

5,6-dihydroxy-indole \_\_\_\_\_ g. 1  
Acetic acid \_\_\_\_\_ cc. 5  
Water to make 100 cc.

Naturally white or nearly white live hair is impregnated with this solution. After contact for 20 minutes, the excess solution is blotted off, for example by means of a towel, and an aqueous solution having the following composition is then applied:

Sodium chloride \_\_\_\_\_ g. 4  
Water \_\_\_\_\_ cc. 100  
20% ammonia \_\_\_\_\_ cc. 17

After contact for 20 minutes, the hair is rinsed clear with water and dried. The hair is dyed a dark grey which gradually changes to black. (This constitutes a progressive dyeing.)

#### Example II

An impregnating solution as set forth in Example I is applied to naturally white live hair.

This solution is left in contact with the hair for 20 minutes, then blotted off, and the following solution is then applied:

Sodium chloride \_\_\_\_\_ g. 4  
Hydrogen peroxide (20 vol.) (6% of  $H_2O_2$ ) \_\_\_\_\_ cc. 2.5  
Water to make 100 cc.

This solution is left in contact with the hair for 1 hour, and the hair is then rinsed, shampooed, rinsed again and dried. A light grey shade is obtained, which remains substantially unchanged in the following weeks.

#### Example III

Almost white live hair is impregnated with an impregnating solution as set forth in Example I. After contact for 20 minutes, the excess solution is blotted off and a second solution having the following composition is then applied:

Sodium chloride \_\_\_\_\_ g. 4  
Water \_\_\_\_\_ cc. 100  
20% ammonia \_\_\_\_\_ cc. 17  
Hydrogen peroxide (20 vol.) (6% of  $H_2O_2$ ) \_\_\_\_\_ cc. 0.3

This second solution is left in contact with the hair for 30 minutes, and the hair is then rinsed, shampooed, rinsed again and dried. The hair is dyed jet-black.

#### Example IV

Almost white live hair is impregnated with an impregnating solution as set forth in Example I.

After contact for 20 minutes, the excess solution is blotted off and the following solution is then applied:

Sodium chloride \_\_\_\_\_ g. 4  
Monomethylamine (in 33% aqueous solution) \_\_\_\_\_ cc. 10  
Hydrogen peroxide (20 vol.) (6% of  $H_2O_2$ ) \_\_\_\_\_ cc. 2.5  
Water to make 100 cc.

This solution is left in contact with the hair for 20 minutes, and the hair is then rinsed, shampooed, rinsed again and dried. The hair is dyed medium ash-blond.

#### Example V

Nearly white live hair is impregnated with an impregnating solution as defined in Example I. After a period of contact of 20 minutes, the excess solution is blotted

off and an aqueous solution having the following composition is applied:

|                                                                    |      |     |
|--------------------------------------------------------------------|------|-----|
| Sodium chloride                                                    | g--  | 2.8 |
| 20% ammonia                                                        | cc-- | 6   |
| Hydrogen peroxide (20 vol.) (6% of H <sub>2</sub> O <sub>2</sub> ) | cc-- | 23  |
| Water to make 100 cc.                                              |      |     |

After contact for 20 minutes, the hair is rinsed, shampooed, rinsed again and dried. A medium brown shade is obtained.

#### Example VI

Naturally white or nearly white hair is impregnated with an impregnating solution as defined in Example I.

The solution is left in contact for 20 minutes, whereafter the excess solution is blotted off and an aqueous solution having the following composition is applied:

|                                                                    |      |     |
|--------------------------------------------------------------------|------|-----|
| Sodium chloride                                                    | g--  | 3.2 |
| 20% ammonia                                                        | cc-- | 2   |
| Hydrogen peroxide (20 vol.) (6% of H <sub>2</sub> O <sub>2</sub> ) | cc-- | 16  |
| Water to make 100 cc.                                              |      |     |

This solution is left in contact with the hair for 20 minutes, the hair is then rinsed, shampooed, rinsed again and dried. A light brown shade is obtained.

#### Example VII

Naturally white live hair is treated with an impregnating solution as defined in Example I.

This solution is left in contact with the hair for 30 minutes, whereafter the excess solution is blotted off and an aqueous solution having the following composition is applied to the hair.

|                                                                    |      |    |
|--------------------------------------------------------------------|------|----|
| Sodium chloride                                                    | g--  | 5  |
| Triethanolamine                                                    | cc-- | 26 |
| Hydrogen peroxide (20 vol.) (6% of H <sub>2</sub> O <sub>2</sub> ) | cc-- | 10 |
| Water                                                              | cc-- | 75 |

After contact for 30 minutes, rinsing, shampooing, rinsing again and drying, the hair is dyed grey.

#### Example VIII

Almost white live hair is impregnated with an impregnating solution as defined in Example I, which is left in contact therewith for 20 minutes. After blotting off the excess solution, the following solution is applied:

|                                                      |      |     |
|------------------------------------------------------|------|-----|
| Sodium chloride                                      | g--  | 4.2 |
| Chloramine T (sodium N-chloro-p-toluen-sulphonamide) | g--  | 1.2 |
| 20% ammonia                                          | cc-- | 14  |
| Water to make 100 cc.                                |      |     |

After contact for 20 minutes, the hair is rinsed, shampooed, rinsed again and dried. The hair is dyed a fine deep black.

#### Example IX

Naturally white live hair is impregnated with the following impregnating solution:

|                       |      |     |
|-----------------------|------|-----|
| 5,6-dihydroxy-indole  | g--  | 1   |
| Acetic acid           | cc-- | 0.5 |
| Water to make 100 cc. |      |     |

The pH-value of this solution is 3.3. This solution is left in contact with the hair for 15 minutes. The excess solution is then blotted off and an aqueous 4% sodium iodate solution is then applied to hair. After 15 minutes, the hair is rinsed, shampooed, rinsed again and dried. A dark grey shade is obtained.

#### Example X

A solution having the following composition is prepared:

|                      |      |     |
|----------------------|------|-----|
| 5,6-dihydroxy-indole | g--  | 1   |
| Water                | cc-- | 100 |

The pH-value of such a solution is 6.2. This solution is applied to naturally white live hair and left in contact

therewith for 15 minutes. After blotting off the excess solution, an aqueous 4% sodium iodate solution is applied to the hair. After this solution has been allowed to act for 15 minutes, the hair is rinsed, shampooed, rinsed again and dried. The hair is dyed a dark grey, which is not, however, as dark as the shade obtained in Example IX.

#### Example XI

Naturally white live hair is treated with an impregnating solution as defined in Example IX.

After contact for 15 minutes, the excess solution is blotted off and an aqueous 4% sodium periodate solution is then applied to the hair. After contact for 15 minutes, rinsing, shampooing, rinsing again and drying, the hair is dyed in a grey shade which is a little lighter than that obtained in Example X.

#### Example XII

A solution having the following composition is prepared:

|                      |      |     |
|----------------------|------|-----|
| 5,6-dihydroxy-indole | g--  | 1   |
| Water                | cc-- | 100 |

This solution is applied to naturally white live hair and, after 15 minutes, the excess liquid is blotted off and an aqueous 4% sodium periodate solution is then applied to the hair. After contact for 15 minutes, the hair is rinsed, shampooed, rinsed again and dried. The hair is dyed a light grey.

#### Example XIII

Hair is impregnated with an impregnating solution as defined in Example IX.

This solution is left in contact with the hair for 15 minutes, whereafter the excess liquid is blotted off and an equal volume of an aqueous 5% sodium persulphate solution is applied thereto. After 15 minutes, the hair is rinsed, shampooed, rinsed again and dried. A medium grey is obtained.

#### Example XIV

An aqueous solution containing 1% by weight of 5,6-dihydroxy-indole is applied to naturally white live hair. This solution is left in contact with the hair for 15 minutes. The excess solution is then blotted off and an aqueous 5% sodium persulphate solution is applied.

After 15 minutes, the hair is rinsed, shampooed, rinsed again and dried. The shade obtained is medium grey.

#### Example XV

Naturally white live hair is impregnated with an impregnating solution as defined in Example I.

When this solution has been allowed to act for 20 minutes, the excess solution is blotted off and a solution having the following composition is applied:

|                       |      |     |
|-----------------------|------|-----|
| 20% ammonia           | cc-- | 15  |
| Sodium iodate         | g--  | 0.5 |
| Water to make 100 cc. |      |     |

After contact for 20 minutes, the hair is rinsed, shampooed, rinsed again and dried. There is obtained a very dark grey shade having a violet tinge, gradually changing to black.

#### Example XVI

Almost white live hair is impregnated with an impregnating solution as defined in Example I which is left in contact therewith for 20 minutes. The excess solution is then blotted off and a solution having the following composition is applied thereto:

|                       |      |     |
|-----------------------|------|-----|
| Sodium periodate      | g--  | 0.5 |
| 20% ammonia           | cc-- | 15  |
| Water to make 100 cc. |      |     |

This solution is allowed to act for 20 minutes and the hair is then rinsed, shampooed, rinsed again, and dried. There is directly obtained a fine black shade, which is substantially permanent.

*Example XVII*

Live, almost white hair is impregnated with an impregnating solution as defined in Example I.

After contact for 20 minutes, the excess liquid is blotted off and a solution having the following composition is applied to the hair:

Ammonium persulphate ----- g 0.5  
20% ammonia ----- cc 15  
Water to make 100 cc.

This solution is left in contact with the hair for 20 minutes. After rinsing, shampooing, rinsing again and drying, the hair is dyed a fine deep black.

*Example XVIII*

A solution having the following composition is employed to impregnate almost white live hair:

5,6-dihydroxy-indole ----- g 1  
Monochloroacetic acid ----- g 1  
Water to make 100 cc.

After contact for 20 minutes with the hair, the excess liquid is blotted off and a solution having the following composition is applied:

Ammonium persulphate ----- g 6  
Sodium chloride ----- g 4  
Monochloroacetic acid ----- g 3  
Water to make 100 cc.

This solution is left in contact with the hair for 20 minutes, whereafter the hair is rinsed, shampooed, rinsed again and dried. The hair is dyed a medium grey.

It is to be understood that the invention includes dead hair or similar material dyed by employing the dyeing process according to the application e.g., hair, bristles, felt, fur and like products so dyed.

## What we claim is:

1. A process for dyeing live human hair and keratinous fibers at room temperature by means of 5,6-dihydroxy-indole which comprises impregnating said materials in a first step with an aqueous solution of said dihydroxy-indole adjusted to a pH value of less than 7 and, after having allowed impregnation to proceed for 5 to 60 minutes and having blotted off the excess solution, applying in a second step onto the impregnated material an aqueous solution containing a nitrogenous base selected from the group consisting of ammonia, basic ammonium salts and organic amines and further containing an oxidizing agent selected from the group consisting of hydrogen peroxide, alkali metal and ammonium bromates, iodates, periodates, perborates and persulphates and alkali metal salts of N-chlorinated sulphonamides.
2. A process for dyeing live human hair and keratinous fibers at room temperature by means of 5,6-dihydroxy-indole which comprises impregnating said materials in a first step with an aqueous solution containing from 0.1% to 10% by weight of 5,6-dihydroxyindole and adjusted to a pH-value of less than 7 and, after having allowed impregnation to proceed for 5 to 60 minutes and blotted off the excess solution, applying in a second step onto the impregnated material an aqueous solution containing a nitrogenous base selected from the group consisting of ammonia, basic ammonium salts and organic amines and further containing an oxidizing agent selected from the group consisting of hydrogen peroxide, alkali metal and ammonium bromates, iodates, periodates, perborates and persulphates and alkali metal salts of N-chlorinated sulphonamides.
3. A process for dyeing live human hair and keratinous fibers at room temperature by means of 5,6-dihydroxy-indole which comprises impregnating said materials in a first step with an aqueous solution containing from 0.1% to 10% by weight of 5,6-dihydroxyindole and adjusted to a pH-value of less than 7 and, after having allowed impregnation to proceed for 5 to 60 minutes and blotted off the excess solution, applying in a second step onto the impregnated material an aqueous solution containing a nitrogenous base selected from the group consisting of ammonia, basic ammonium salts and organic amines and further containing an oxidizing agent selected from the group consisting of hydrogen peroxide, alkali metal and ammonium bromates, iodates, periodates, perborates and persulphates and alkali metal salts of N-chlorinated sulphonamides.

## References Cited in the file of this patent

## UNITED STATES PATENTS

1,133,594 Monsavon Nov. 19, 1956

UNITED STATES PATENT OFFICE  
CERTIFICATE OF CORRECTION

Patent No. 2,934,396

April 26, 1960

Roger Charle et al.

It is hereby certified that error appears in the printed specification of the above numbered patent requiring correction and that the said Letters Patent should read as corrected below.

Column 8, line 35, list of References Cited, strike out "UNITED STATES PATENTS" and insert instead -- FOREIGN PATENT --; line 36, strike out "Monsavon" and insert instead -- France --.

Signed and sealed this 25th day of October 1960.

(SEAL)

Attest:

KARL H. AXLINE  
Attesting Officer

ROBERT C. WATSON  
Commissioner of Patents